

## UNITED STATES PATENT OFFICE

RICHARD W. LEWIS, OF MONTCLAIR, NEW JERSEY

EMULSIONS AND MATERIALS, METHODS AND PROCESSES FOR THE PREPARATION  
THEREOF

No Drawing.

Application filed July 5, 1924. Serial No. 724,291.

My present invention relates to dispersions and to processes and methods of preparing them. It relates particularly to dispersions such as those of bituminous material in water, to dispersing agents, to grinding and shredding agents for the disperse media, and to methods and processes of using said agents for preparing the dispersions, and is applicable in the arts generally.

5 In the dispersion of asphalt, for example, in water, materials such as clay are generally used which have the property of shredding or disintegrating the material to be dispersed when they are mechanically stirred together 10 in the dispersing medium, in addition to the property of causing the one to be dispersed in the other. There are, however, certain agents which are effective in holding the disperse medium in suspension in the dispersing 15 medium when the former is presented in a sufficiently finely divided state but which by their nature or by reason of the proportions in which they are used are ineffective in themselves, to grind or shred the disperse medium 20 so that it may be dispersed.

25 I have discovered, however, that by saturating or impregnating a bed or slip of an inert finely divided grinding material with a dispersing agent of the last mentioned nature and mechanically stirring the material to be dispersed thereinto, the inert material tears or sheds the latter, and the dispersing agent then becomes effective to disperse it, and to maintain it in dispersion, the dispersing medium in such case being usually applied as the liquid is mixed with the grinding material to make a slip therewith. In the grinding action any tendency of the dispersing agent to serve as a grinder or disintegrator of the disperse medium is added to the effective tendency of the inert grinder. In some cases, however, though either the inert grinder or the dispersing agent alone may not have an effective grinding tendency, 35 I can select and use such of these as when taken and used together will have a resultant effective grinding and dispersing action.

An example of an effective grinding material incapable of maintaining a dispersion is 40 200-mesh powdered silica, and of a dispers-

ing agent for use therewith is aluminum hydroxide; or a hydrosol. The impregnation of a grinding bed or slip such as of fine silica and water with such a mixture and the stirring thereinto of an asphalt, would result in 55 the dispersion of the asphalt in water.

It is then an object of my invention to provide a dispersing mixture or slip comprising an inert finely divided grinding material and a dispersing agent which by its nature 60 or by reason of the proportions in which it is used is incapable in itself of shredding the material to be dispersed but which is effective in holding the disperse material in dispersion when it is presented to it in a sufficiently 65 finely divided state.

It is further an object of my invention to provide methods and processes for grinding and disintegrating the material to be dispersed and producing a dispersion thereof 70 in the dispersing medium.

Other objects of my invention will appear from the specification.

As grinding material I use finely divided material which is harder than the material 75 to be dispersed, such as silica, slate dust, etc. For most purposes I employ such a powder which is also insoluble so as to avoid blooming thereof after the emulsion has been put in use and the dispersing medium removed as in 80 the application of a bitumen emulsion in water in which the water dries out and the bitumen hardens into a resistant covering.

85 Suitable dispersing agents I find to be for example tannic acid, soap, basic sulphates of copper or of iron, aluminum hydroxide, ferric hydroxide, insoluble phosphate such for example as chemicals having empirical formulas of  $R''' PO_4$  and  $R''_3 (PO_4)_2$ , ferric or aluminum oxides and hydrates, hydrosols and 90 hydrogels of substances normally insoluble, etc. By the term hydrate, as for example aluminum hydrate, I intend any hydrate inclusive of the hydrosols, hydrogels, gelatinous precipitates, or normal hydroxides.

95 For dispersing media I use any substance in the liquid state which may be found desirable for such use, and for the dispersed material I use bituminous material, waxes, pitches, gums, etc., such as stearin pitch, the 100

asphalts, gilsonite, paraffin, gutta percha, caoutchouc, etc.

In the use of the processes, methods, and materials of my invention I perform the following operation or operations, a bituminous emulsion in water being used as an example.

A mixture of finely divided material such as 900 lbs. of silica, 200 lbs. of aluminum hydroxide, and water is agitated in a mechanical mixer while 9000 lbs. of a bitumen in the liquid or semi-liquid state is added. The proportions given are those used in shop practice to produce one useful dispersion, but other useful dispersions, of course, have been obtained by varying the relative proportions to meet varying conditions of service of the material, and such dispersions are within the scope of my invention. The silica serves as a mechanical grinder and shredder for the bitumen while the aluminum hydroxide serves as an emulsifying agent with the result that the bitumen is dispersed in the water.

The grinding base according to my invention is used in the emulsion as a filler when desired; or when desired it is separated centrifugally or settled out as by diluting the emulsion with sufficient additional dispersing medium or other medium for that purpose and used over again. In some cases I make the dispersing process and the settling or separating process to follow each other cyclically as parts or steps of a continuous process.

After once having started the shredding and grinding and dispersing of the material to be dispersed, I can in some cases continue the process with the addition of only the material to be dispersed, the dispersing medium, and the dispersing agent, because after active grinding has once been started the shredding tendency of the dispersion will be sufficient to continue the shredding. In other cases in such a continuous process it is necessary to add the grinding material in considerably lessened amounts only.

The dispersions may be qualified, depending upon the use to which they are to be put, by the addition of a material which is soluble or miscible in the dispersing medium, is volatile, and which has little or no solvent effect on the dispersed material such as denatured alcohol in an asphalt-water dispersion for reducing the freezing point of the dispersion or dispersing medium to thereby permit the shipping and use of the dispersion in freezing weather. This material I add during or after the dispersing operation.

I have discovered that when the paint pigments of commerce, such as the iron oxides, chrome-green, and others, are utilized as dispersing agents that they produce stable dispersions and have the desirable property in such dispersions of irreversibility. Further-

more, all or certain of these materials will function better as dispersing agents if one or more of the more active dispersing agents such as mentioned above are utilized in the process of production of the dispersion. In this way simple dispersions, or complex dispersions, as may be desired, are produced at the will of the operator, and at the same time the desirable feature is available of pre-determining the color of the finished dispersion by selecting as the dispersing agent or as one of the dispersing agents that oxide or other pigment giving the desired color.

The subject matter of invention disclosed in this application is disclosed and/or claimed in the following copending applications of Richard W. Lewis, to wit: Serial No. 33,804, filed May 27, 1925 (Patent No. 1,787,418); Serial No. 491,968, filed Oct. 29, 1930; and Serial No. 491,969, filed Oct. 29, 1930.

I claim:

A dispersion of bitumen in water comprising a bitumen, water and a mixture for preparing and maintaining the dispersion, comprising an element of the group consisting of silica and slate dust and an element of the group consisting of tannic acid and soap.

In testimony whereof I hereto affix my signature.

RICHARD W. LEWIS.

95

100

105

110

115

120

125

130

## UNITED STATES PATENT OFFICE

RICHARD W. LEWIS, OF MONTCLAIR, NEW JERSEY

## DISPERSIONS AND THE PRODUCTION THEREOF

No Drawing.

Application filed October 29, 1930. Serial No. 491,968.

My present invention relates to dispersions and to processes and methods of preparing them. It relates particularly to dispersions such as those of bituminous material in water, to dispersing agents, to grinding and shredding agents for the disperse media, and to methods and processes of using said agents for preparing the dispersions, and is applicable in the arts generally.

In the dispersion of asphalt, for example, in water, materials such as clay are generally used which have the property of shredding or disintegrating the material to be dispersed when they are mechanically stirred together in the dispersing medium, in addition to the property of causing the one to be dispersed in the other. There are, however, certain agents which are effective in holding the disperse medium in suspension in the dispersing medium when the former is presented in a sufficiently finely divided state but which by their nature or by reason of the proportions in which they are used are ineffective in themselves, to grind or shred the disperse medium so that it may be dispersed.

I have discovered, however, that by saturating or impregnating a bed or slip of an inert finely divided grinding material with a dispersing agent of the last mentioned nature and mechanically stirring the material to be dispersed thereinto, the inert material tears or shreds the latter, and the dispersing agent then becomes effective to disperse it, and to maintain it in dispersion, the dispersing medium in such case being usually applied as the liquid is mixed with the grinding material to make a slip therewith. In the grinding action any tendency of the dispersing agent to serve as a grinder or disintegrator of the disperse medium is added to the effective tendency of the inert grinder. In some cases, however, though either the inert grinder or the dispersing agent alone may not have an effective grinding tendency, I can select and use such of these as when taken and used together will have a resultant effective grinding and dispersing action.

An example of an effective grinding material incapable of maintaining a dispersion

is 200-mesh powdered silica, and of a dispersing agent for use therewith is aluminum hydroxide or a hydrosol. The impregnation of a grinding bed or slip such as of fine silica and water with such a mixture and the stirring thereinto of an asphalt, would result in the dispersion of the asphalt in water.

It is then an object of my invention to provide a dispersing mixture or slip comprising an inert finely divided grinding material and a dispersing agent which by its nature or by reason of the proportions in which it is used is incapable in itself of shredding the material to be dispersed but which is effective in holding the disperse material in dispersion when it is presented to it in a sufficiently finely divided state.

It is further an object of my invention to provide methods and processes for grinding and disintegrating the material to be dispersed and producing a dispersion thereof in the dispersing medium.

Other objects of my invention will appear from the specification.

As grinding material I use finely divided material which is harder than the material to be dispersed, such as silica, slate dust, barytes, marble dust and other forms of powdered calcite, fibrous talc, and various artificial preparations such as the zinc oxide pigment of commerce and precipitated barium sulphate.

In fact, for the intended purpose there may be used most of the insoluble inorganic substances such, for example, as the class of substances known as mineral fillers and which are readily obtainable commercially in suitable powdered form, provided only that the pulverization of the material has been carried far enough to permit of its forming a paste or mud when mixed with water but has not been carried far enough so that the individual particles are capable of acting as true emulsifying agents. From such a classification I exclude clay and other so-called colloidal materials whose subdivision cannot be arrested at will. Such materials are excluded because of the fact that it is difficult, if not impossible, to arrest the prog-